# EUROPEAN PATENT SPECIFICATION

(11) **EP 4 433 568 B1**
(45) Date of publication and mention of the grant of the patent: **26.02.2025**
(21) Application number: 22808999.1
(22) Date of filing: 20.10.2022
(51) Int. Cl.: C11D 1/29, C11D 17/00

(54) **DETERGENT COMPOSITIONS**
WASCHMITTELZUSAMMENSETZUNGEN
COMPOSITIONS DÉTERGENTES

(30) Priority: 21.10.2021 EP 21203922; 21.10.2021 EP 21203927; 21.10.2021 EP 21203931
(43) Date of publication of application: 25.09.2024
(73) Proprietor: Unilever IP Holdings B.V., 3013 AL Rotterdam (NL); Unilever Global IP Limited, Wirral, Merseyside CH62 4ZD (GB)
(72) Inventor: BURNHAM, Neil Stephen, 6708 WH Wageningen (NL); GRAINGER, David Stephen, 6708 WH Wageningen (NL); THORLEY, David Christopher, 6708 WH Wageningen (NL)
(74) Representative: McHugh, Paul Edward
(86) International application number: PCT/EP2022/079231
(87) International publication number: WO 2023/067074

(56) References cited:
- EP-A2- 0 339 426
- CA-A1- 2 067 789
- CN-A- 1 470 316
- CN-A- 109 134 843
- GB-A- 1 068 528
- GB-A- 1 135 136
- JP-A- 2002 327 194
- JP-A- H0 472 395
- US-A- 4 412 944
- US-A1- 2014 309 155
- US-B1- 6 172 022
- MARY AM LIEBERT: "Final Report on the Safety Assessment of Sodium Myreth Sulfate", JOURNAL OF THE AMERICAN COLLEGE OF TOXICOLOGY, vol. 11, no. 1, 1 January 1992 (1992-01-01), US, pages 157 - 163, XP055905478, ISSN: 0730-0913, DOI: 10.3109/10915819209141996
- ANONYMOUS: "Sodium myreth sulfate", WIKIPEDIA, THE FREE ENCYCLOPEDIA, 29 May 2020 (2020-05-29), XP055905958, Retrieved from the Internet <URL:https://en.wikipedia.org/w/index.php?title=Sodium_myreth_sulfate&oldid=959579286> [retrieved on 20220328]

## Description

### Field of the Invention

The invention relates to the field of detergent compositions, in particular liquid detergent compositions. The compositions are particularly useful for the washing of the items in the home, including dishes, cutlery and other cooking and eating utensils, for laundry of clothes and for the washing of the body including the hair. The compositions of the invention are particularly useful in the field of home care, for example in laundry compositions and hand dish wash compositions.

### Background of the Invention

One common class of anionic surfactant used are Alkyl Ether Sulphates (AES). The generic structure for the sodium salt is:

Where, on average n is ~1-3 and n is 10-13.

In practice the materials used in laundry and dish wash products contain of a mixture of materials with a distribution of values for both n and r. A common commercial material is sodium C12/C14 3EO sulfate. Liquid detergent composition comprising alkyl ethoxylate sulfate of specific distribution of ethoxylated material is disclosed in JP H04 72395. A method to produce readily thickenable C12/14 alkyl ethoxylate sulfate surfactant in liquid detergent composition is disclosed in CA 2 067 789. These materials generally require assistance to produce the required viscosity of the target composition, for example by including large amounts of salt, or other viscosity modifiers.

We have surprising found that by specifying an amount of the total of C14 material, and by specifying the distribution of the ethoxylated materials, then the viscosity of the resulting composition is much higher, hence the level of salt or other viscosity modifiers can be reduced considerably, or even such modifiers may not be necessary.

### Summary of the Invention

The invention relates in a first aspect to a liquid detergent composition comprising:
from 2 to 25 wt.% of a C12-C14 alkyl ethoxylated sulfate surfactant;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24
wt.%, the level of 3EO is from 20 to 35 wt.%, and the level of 4EO is from 12 to 25 wt.%; and, wherein the C12-C14 alkyl ethoxylated sulfate surfactant includes at most 10 wt.% alkyl chains of C15 and higher.

The alkyl ethoxylated sulfate surfactant comprises a C14 alkyl group at a level of at least 70 wt.%, even more preferably at least 75 wt.%, even more preferably at least 80 wt.%, even more preferably at least 85 wt.%, even more preferably at least 90 wt.%, even more preferably at least 95 wt.% of the alkyl ethoxylated sulfate surfactant.

The alkyl ethoxylated sulfate surfactant is present at a level of from 2 to 25 wt.%, most preferably from 2.5 to 20 wt.%.

Preferably the average degree of ethoxylation (EO) of the alkyl ethoxylated sulfate surfactant is from 2.7 to 3.3.

With reference to the wt.% of the total ethoxylated portion of said alkyl ethoxylated sulfate surfactant, the level of 1EO is from 12 to 23 wt.%, preferably from 13 to 22 wt.%, more preferably from 14 to 21 wt.%, even more preferably from 15 to 20 wt.%.

Preferably with reference to the wt.% of the total ethoxylated portion of said alkyl ethoxylated sulfate surfactant, the level of 2EO is from 16 to 23 wt.%, preferably from 17 to 22 wt.%, more preferably from 18 to 22 wt.%.

Preferably with reference to the wt.% of the total ethoxylated portion of said alkyl ethoxylated sulfate surfactant, the level of 3EO is from 20 to 30 wt.%, preferably from 21 to 28 wt.%, more preferably from 22 to 26 wt.%.

Preferably with reference to the wt.% of the total ethoxylated portion of said alkyl ethoxylated sulfate surfactant, the level of 4EO is from 13 to 24 wt.%, preferably from 14 to 22 wt.%, more preferably from 15 to 21 wt.%.

Preferably the detergent composition additionally comprises from 1 to 40 wt.%, preferably from 2 to 30 wt.%, more preferably from 4 to 25 wt.%, most preferably from 5 to 20 wt.% of one or more other surfactants (other than the specified alkyl ethoxylated sulfate surfactant) selected from anionic surfactants, nonionic surfactants, cationic surfactants and amphoteric surfactants, preferably anionic surfactants, nonionic surfactants and amphoteric surfactants.

Preferably the detergent composition is a laundry liquid detergent composition or a liquid hand dish wash composition, more preferably an aqueous liquid detergent composition, more preferably an aqueous laundry liquid detergent composition or an aqueous liquid hand dish wash composition.

In a second aspect, the invention relates to the use of a C12-C14 alkyl ethoxylated sulfate surfactant to increase the viscosity of a liquid detergent composition;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5; and,
wherein with reference to the wt.% of the total ethoxylated portion of said alkyl ethoxylated sulfate surfactant, the level of 1EO is from 12 to 23 wt.%, the level of 2EO is from 15 to 24
wt.%, the level of 3EO is from 20 to 35 wt.%, and the level of 4EO is from 12 to 25 wt.%; and, wherein the C12-C14 alkyl ethoxylated sulfate surfactant includes at most 10 wt.% alkyl chains of C15 and higher.

In a third aspect, the invention relates to a method to increase viscosity of a liquid detergent composition, wherein said method involves inclusion of 2 to 25 wt.% of a C12-C14 alkyl ethoxylated sulfate surfactant;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24
wt.%, the level of 3EO is from 20 to 35 wt.%, and the level of 4EO is from 12 to 25 wt.%; and, wherein the C12-C14 alkyl ethoxylated sulfate surfactant includes at most 10 wt.% alkyl chains of C15 and higher.

Preferably, in said use or method, the increased viscosity is measured in reference to a constant salt level, preferably NaCl, in said detergent composition.

### Detailed Description of the Invention

### Alkyl ethoxylated sulfate surfactant

The detergent composition comprises from 2 to 25 wt.% of a C12-C14 alkyl ethoxylated sulfate surfactant;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24
wt.%, the level of 3EO is from 20 to 35 wt.%, and the level of 4EO is from 12 to 25 wt.%; and, wherein the C12-C14 alkyl ethoxylated sulfate surfactant includes at most 10 wt.% alkyl chains of C15 and higher (e.g. C16, C18, C20, C22 etc).

The C12-C14 alkyl ethoxylated sulfate surfactant includes at most 10 wt.%, more preferably 8 wt.%, even more preferably 6 wt.%, even more preferably 5 wt.%, even more preferably 4 wt.%, even more preferably 3 wt.%, even more preferably 2 wt.%, most preferably 1 wt.% alkyl chains of C15 and higher. Even more preferably the C12-C14 material is free from alkyl chains of C15 and higher (e.g. C16, C18, C20, C22 etc).

Preferably the C12-C14 alkyl ethoxylated sulfate surfactant comprises 90 to 100 wt.%, preferably from 91 to 100 wt.%, more preferably from 92 to 100 wt.%, more preferably from 93 to 100 wt.%, more preferably from 94 to 100 wt.%, more preferably from 95 to 100 wt.%, more preferably from 96 to 100 wt.%, more preferably from 97 to 100 wt.%, more preferably from 98 to 100 wt.%, more preferably from 99 to 100 wt.% of C12 and C14 alkyl chains.

The claimed alkyl ethoxylated sulfate surfactant is present at a level of from 2 to 25 wt.%, most preferably from 2.5 to 20 wt.%.

The claimed alkyl ethoxylated sulfate surfactant has an average degree of ethoxylation (EO) of from 2.5 to 3.5, preferably from 2.7 to 3.3.

The average degree of ethoxylation of the alkyl ethoxylated sulfate surfactant of from 2.5 to 3.5, preferably from 2.7 to 3.3. This average value is calculated based on the levels of all of the different ethoxylated material (1EO, 2EO, 3EO, 4EO, 5EO etc...) present on the surfactant. To be clear, the level of 0EO surfactant (the non-ethoxylated portion of the surfactant) is not included in the calculation of the average degree of ethoxylation.

It is understood that it is common that there is a non-ethoxylated portion of alkyl sulfate surfactant also present in these surfactant mixtures. For example, after the ethoxylation process, the resulting material is a mixture of 0EO, 1EO, 2EO, 3EO, 4EO, 5EO etc... materials. It is a mixture of ethoxylated material of various EO, with some non-ethoxylated material.

It is preferred that the wt.% level of non-ethoxylated material in the alkyl ethoxylated sulfate surfactant is from 8 to 27 wt.%, preferably from 10 to 25 wt.%, more preferably from 12 to 22 wt.%. This is calculated based on the wt.% level of non-ethoxylated material with reference to the total amount of alkyl ethoxylated sulfate surfactant.

This preferred level of 0EO material (non-ethoxylated material) in the alkyl ethoxylated sulfate surfactant is different to the levels of 0EO seen in common commercial materials. For example, a common commercial C12-C14 3EO SLES was measured and had a level of 0EO being ~37 wt.% of the total surfactant.

Preferably the alkyl ethoxylated sulfate surfactant comprises a C14 alkyl group at a level of at least 55 wt.%, preferably at least 60 wt.%, more preferably at least 65 wt.%, even more preferably at least 70 wt.%, even more preferably at least 75 wt.%, even more preferably at least 80 wt.%, even more preferably at least 85 wt.%, even more preferably at least 90 wt.%, even more preferably at least 95 wt.% of the alkyl ethoxylated sulfate surfactant. The surfactant may even be composed of C14 alkyl group (i.e., be 100 wt.% C14 alkyl).

While the alkyl group of the alkyl ethoxylated sulfate surfactant may be linear or branched, preferably the alkyl group of alkyl ethoxylated sulfate surfactant is linear.

With reference to the wt.% of the total ethoxylated portion of said alkyl ethoxylated sulfate surfactant, the level of 1EO is from 12 to 23 wt.%, preferably from 13 to 22 wt.%, more preferably from 14 to 21 wt.%, even more preferably from 15 to 20 wt.%.

Preferably with reference to the wt.% of the total ethoxylated portion of said alkyl ethoxylated sulfate surfactant, the level of 2EO is from 16 to 23 wt.%, preferably from 17 to 22 wt.%, more preferably from 18 to 22 wt.%.

Preferably with reference to the wt.% of the total ethoxylated portion of said alkyl ethoxylated sulfate surfactant, the level of 3EO is from 20 to 30 wt.%, preferably from 21 to 28 wt.%, more preferably from 22 to 26 wt.%.

Preferably with reference to the wt.% of the total ethoxylated portion of said alkyl ethoxylated sulfate surfactant, the level of 4EO is from 13 to 24 wt.%, preferably from 14 to 22 wt.%, more preferably from 15 to 21 wt.%.

These preferred features (the wt.% levels of 1EO, 2EO, 3EO and 4EO with reference to the total wt.% of the ethoxylated portion of the alkyl ethoxylated sulfate surfactant) are calculated on the basis of the total level of only the ethoxylated material contained in the surfactant, not including the wt.% portion of the non-ethoxylated material of the surfactant.

For example, the calculation for the level of 1EO would be as follows:
Wt.% of 1EO surfactant ÷ (total wt.% of all ethoxylated portions of the surfactant)

It is understood that it is common that there is a non-ethoxylated portion of alkyl sulfate surfactant also present. This material is not included in the above calculations for the preferred levels of 1EO, 2EO, 3EO and 4EO.

### Methods of Ethoxylation

Ethoxylation reactions are described in Non-Ionic Surfactant Organic Chemistry (N. M. van Os ed), Surfactant Science Series Volume 72, CRC Press.

Preferably the ethoxylation reactions are base catalysed using NaOH, KOH, or NaOCH₃. Even more preferred are catalyst which provide narrower ethoxy distribution than NaOH, KOH, or NaOCH₃. Preferably these narrower distribution catalysts involve a Group II base such as Ba dodecanoate; Group II metal alkoxides; Group II hyrodrotalcite as described in WO 2007/147866. Lanthanides may also be used.

### Specific methods of narrow range ethoxylation

Narrow range ethoxylation catalyst are described in EP3289790 (Procter & Gamble), EP1747183 (Hacros); Santacesatia et al Ind. Eng. Chem. Res. 1992, 31, 2419-2421; US4239917 (Conoco); Li et al ACS Omega. 2021 Nov 9; 6(44): 29774-29780; Hreczuch et al J. Am. Oil Chem. Soc. 1996, 73, 73-78. Catalysts based on Ca or Ba are preferred, most preferably in combination with sulfuric acid.

### General example method

A calcium catalyst was prepared according to EP1747183, with the following composition: n-Butanol 73.5 wt.%, calcium hydroxide 15.2 wt. %, 2-ethylhexanoic acid, and 3.5 wt.%, conc. sulfuric acid 7.8 wt.%.

To prepare the catalyst, a three-neck round bottom flask is equipped with a magnetic stir bar, a glass stopper, a Dean-Stark trap filled with n-butanol, a condenser topped with a calcium chloride drying tube, and is placed in an oil bath. The n-butanol is charged to the flask and. stirring is initiated. The calcium hydroxide is slowly added, and allowed to stir for 15 minutes. A carboxylic acid (such as 2-ethylhexanoic acid) is then added to the mixture via syringe. The flask containing the mixture is then heated to above 120 degrees centigrade at atmospheric pressure. The stirring suspension is allowed to reflux for up to about 8 hours. Under these conditions, water and the dispersing medium will be removed during the process, but the dispersing medium is recycled into the reaction vessel. After cooling to room temperature, the stir bar is removed, and an overhead stirrer is added. The Dean-Stark trap, condenser, drying tube, oil bath, and stoppers are removed. A source of nitrogen, thermometer, water bath, and pressure equalizing dropping funnel are added. The pressure equalizing dropping funnel is charged with an inorganic acid (such as sulfuric acid), and the acid is added over the course of about 3 hours. The internal temperature is maintained at or below about 25 degrees centigrade by the use of a water bath and ice. After the acid is added completely, the suspension is allowed to stir for an additional 30-60 minutes at a temperature of about 25°C

This catalyst was used to produce narrow range ethoxylates as follows:-915 g of a C12-C14 alcohol (C12 = 10 wt.%, C14 = 89 wt.% C16 = 1 wt.%) was charged into a 2 gallon stainless steel autoclave equipped with an overhead stirrer, internal steam heating, water cooling, and thermocouple. The C12-C14 alcohol was vacuum dried at 90°C, then 2.1 g of catalyst was added and vacuum stripped at 90°C until all the solvent was removed (~ 5minutes). The reactor was heated to 140°C and ethylene oxide slowly added. After an induction period a small exothermic reaction is observed on which the addition of ethylene oxide is continued at a pressure of 2 bar, until 3 moles of ethylene oxide in total had been consumed. Temperature was controlled using water cooling and allowed to reach 180°C. When a mole ratio of 3:1 ethylene oxide to C12-C14 alcohol had reacted to form alcohol ethoxylate the temperature was lowered to 90°C and the product vacuumed stripped for 3 hours.

The ethoxylation procedure was repeated using a (C₁₁H₂₃COO)₂Ba described in Ind. Eng. Chem. Res. 1992, 31, 2419-2421 and a barium oxide/sulfuric acid catalyst as described in WO2012028435 (Kolb).

### Sulfation

The alcohol/ethoxylate mixtures may be sulfated by any of the known methods for sulfating such materials (cf. J. Falbe (ed.), "Surfactants in Consumer Products", Springer Verlag, Berlin-Heidelberg, 1987, page 61), preferably using reactors operating on the falling-film principle.

Suitable sulfonating agents are chlorosulfonic acid and, in particular, gaseous sulfur trioxide. The sulfur trioxide is normally diluted with an inert gas, preferably air or nitrogen, and used in the form of a gas mixture containing the sulfonating agent in a concentration of 1 to 8% by volume and, more particularly, 2 to 5% by volume.

The molar ratio of alcohol/ethoxylate mixture to sulfating agent is normally from 1:0.95 to 1:1.3 and is preferably from 1:1 to 1:1.05. The sulfation reaction is normally carried out at temperatures of from 25° to 70° C.

A further reference for the general method for sulfation is Anionic Surfactants Organic Chemistry, Surfactant Science Series 56, Edited by H.W. Stache (Marcel Dekker 1996).

Preferably ether sulfate is produced using SO₃ for the sulfation, preferably in a multitube falling film reactor and that dioxane are reduced to less than 20ppm, more preferably less than 10ppm, most preferably less than 5ppm on a 100% active basis. Methods to reduce dioxane are described in WO2017/179026 (Ballestra) and WO2014/058791 (Chemithon).

### Liquid Detergent

The detergent composition is a liquid detergent composition. Preferably it is an aqueous liquid detergent composition. Such compositions may include water at a level of from 20 to 90 wt.%, preferably 30 to 90 wt.%, more preferably from 40 wt.% to 90 wt.%, most preferably from 50 to 90 wt.%.

### Additional Preferred Ingredients

### Surfactants

Preferably the detergent composition additionally comprises from 1 to 40 wt.%, preferably from 2 to 30 wt.%, more preferably from 4 to 25 wt.%, most preferably from 5 to 20 wt.% of one or more other surfactants (other than the specified alkyl ethoxylated sulfate surfactant) selected from anionic surfactants, nonionic surfactants, cationic surfactants and amphoteric surfactants, preferably anionic surfactants, nonionic surfactants and amphoteric surfactants.

Preferably the additional anionic surfactant is preferably selected from primary alkyl sulfates, linear alkyl benzene sulfonates, internal olefin sulfonates, alpha olefin sulfonates, soaps, anionically modified APGs, furan based anionics and, citrems, tatems and datems, more preferably selected from primary alkyl sulfates, linear alkyl benzene sulfonates, furan based anionics. Most preferred additional anionic surfactants are linear alkyl benzene sulfonates.

Preferably the nonionic surfactant is selected from alcohol alkoxylates (preferably alcohol ethoxylates), alkyl polyglucosides, alkyl polypentosides. Most preferred nonionic surfactants are preferably selected from alcohol ethoxylates having from C12-C15 with a mole average of from 5 to 9 ethoxylates and/or alcohol ethoxylates having from C16-C18 with a mole average of from 5 to 14 ethoxylates.

Preferred amphoteric surfactants include coco amidopropyl betaine (CAPB).

### Further Ingredients

The formulation may contain further ingredients.

If the detergent composition is an aqueous liquid laundry detergent it is preferred that mono propylene glycol or glycerol is present at a level from 1 to 30 wt.%, most preferably 2 to 18 wt.%.

### Fluorescent Agent

The composition preferably comprises a fluorescent agent (optical brightener).

Fluorescent agents are well known and many such fluorescent agents are available commercially. Usually, these fluorescent agents are supplied and used in the form of their alkali metal salts, for example, the sodium salts.

The total amount of the fluorescent agent or agents used in the composition is generally from 0.0001 to 0.5 wt.%, preferably 0.005 to 2 wt.%, more preferably 0.01 to 0.1 wt.%.

Preferred classes of fluorescer are: Di-styryl biphenyl compounds, e.g. Tinopal (Trade Mark) CBS-X, Di-amine stilbene di-sulphonic acid compounds, e.g. Tinopal DMS pure Xtra and Blankophor (Trade Mark) HRH, and Pyrazoline compounds, e.g. Blankophor SN.

Preferred fluorescers are fluorescers with CAS-No 3426-43-5; CAS-No 35632-99-6; CAS-No 24565-13-7; CAS-No 12224-16-7; CAS-No 13863-31-5; CAS-No 4193-55-9; CAS-No 16090-02-1; CAS-No 133-66-4; CAS-No 68444-86-0; CAS-No 27344-41-8.

Most preferred fluorescers are: sodium 2 (4-styryl-3-sulfophenyl)-2H-napthol[1,2-d]triazole, disodium 4,4'-bis{[(4-anilino-6-(N methyl-N-2 hydroxyethyl) amino 1,3,5-triazin-2-yl)]amino}stilbene-2-2' disulphonate, disodium 4,4'-bis{[(4-anilino-6-morpholino-1,3,5-triazin-2-yl)]amino} stilbene-2-2' disulphonate, and disodium 4,4'-bis(2-sulphostyryl)biphenyl.

### Shading dye

It is advantageous to have shading dye present in the formulation.

Dyes are described in Color Chemistry Synthesis, Properties and Applications of Organic Dyes and Pigments, (H Zollinger, Wiley VCH, Zürich, 2003) and, Industrial Dyes Chemistry, Properties Applications. (K Hunger (ed), Wiley-VCH Weinheim 2003).

Dyes for use in laundry detergents preferably have an extinction coefficient at the maximum absorption in the visible range (400 to 700nm) of greater than 5000 L mol⁻¹ cm⁻¹, preferably greater than 10000 L mol⁻¹ cm⁻¹.

Preferred dye chromophores are azo, azine, anthraquinone, phthalocyanine and triphenylmethane. Azo, anthraquinone, phthalocyanine and triphenylmethane dyes preferably carry a net anionic charged or are uncharged. Azine dyes preferably carry a net anionic or cationic charge.

Blue or violet Shading dyes are most preferred. Shading dyes deposit to fabric during the wash or rinse step of the washing process providing a visible hue to the fabric. In this regard the dye gives a blue or violet colour to a white cloth with a hue angle of 240 to 345, more preferably 260 to 320, most preferably 270 to 300. The white cloth used in this test is bleached non-mercerised woven cotton sheeting.

Shading dyes are discussed in WO 2005/003274, WO 2006/032327 (Unilever), WO 2006/032397 (Unilever), WO 2006/045275 (Unilever), WO 2006/027086 (Unilever), WO 2008/017570 (Unilever), WO 2008/141880 (Unilever), WO 2009/132870 (Unilever), WO 2009/141173 (Unilever), WO 2010/099997 (Unilever), WO 2010/102861 (Unilever), WO 2010/148624 (Unilever), WO 2008/087497 (P&G), WO 2011/011799 (P&G), WO 2012/054820 (P&G), WO 2013/142495 (P&G), WO 2013/151970 (P&G), WO 2018/085311 (P&G) and WO 2019/075149 (P&G).

A mixture of shading dyes may be used.

The shading dye chromophore is most preferably selected from mono-azo, bis-azo and azine.

Mono-azo dyes preferably contain a heterocyclic ring and are most preferably thiophene dyes. The mono-azo dyes are preferably alkoxylated and are preferably uncharged or anionically charged at pH=7. Alkoxylated thiophene dyes are discussed in WO2013/142495 and WO2008/087497. A preferred example of a thiophene dye is shown below:

Bis-azo dyes are preferably sulphonated bis-azo dyes. Preferred examples of sulphonated bis-azo compounds are direct violet 7, direct violet 9, direct violet 11, direct violet 26, direct violet 31, direct violet 35, direct violet 40, direct violet 41, direct violet 51, direct violet 66, direct violet 99 and alkoxylated versions thereof.

Alkoxylated bis-azo dyes are discussed in WO2012/054058 and WO/2010/151906.

An example of an alkoxylated bis-azo dye is :

Azine dyes are preferably selected from sulphonated phenazine dyes and cationic phenazine dyes. Preferred examples are acid blue 98, acid violet 50, dye with CAS-No 72749-80-5, acid blue 59, and the phenazine dye selected from: wherein:
X₃ is selected from: -H; -F; -CH₃; -C₂H₅; -OCH₃; and, -OC₂H₅;
X₄ is selected from: -H; -CH₃; -C₂H₅; -OCH₃; and, -OC₂H₅;
Y₂ is selected from: -OH; -OCH₂CH₂OH; -CH(OH)CH₂OH; -OC(O)CH₃; and, C(O)OCH₃. Anthraquinone dyes covalently bound to ethoxylate or propoxylated polyethylene imine may be used as described in WO2011/047987 and WO 2012/119859.

The shading dye is preferably present is present in the composition in range from 0.0001 to 0.1wt %. Depending upon the nature of the shading dye there are preferred ranges depending upon the efficacy of the shading dye which is dependent on class and particular efficacy within any particular class. As stated above the shading dye is preferably a blue or violet shading dye.

### Perfume

The composition preferably comprises a perfume. Many suitable examples of perfumes are provided in the CTFA (Cosmetic, Toiletry and Fragrance Association) 1992 International Buyers Guide, published by CFTA Publications and OPD 1993 Chemicals Buyers Directory 80th Annual Edition, published by Schnell Publishing Co.

Preferably the perfume comprises at least one note (compound) from: alpha-isomethyl ionone, benzyl salicylate; citronellol; coumarin; hexyl cinnamal; linalool; pentanoic acid, 2-methyl-, ethyl ester; octanal; benzyl acetate; 1,6-octadien-3-ol, 3,7-dimethyl-, 3-acetate; cyclohexanol, 2-(1,1-dimethylethyl)-, 1-acetate; delta-damascone; beta-ionone; verdyl acetate; dodecanal; hexyl cinnamic aldehyde; cyclopentadecanolide; benzeneacetic acid, 2-phenylethyl ester; amyl salicylate; beta-caryophyllene; ethyl undecylenate; geranyl anthranilate; alpha-irone; beta-phenyl ethyl benzoate; alpa-santalol; cedrol; cedryl acetate; cedry formate; cyclohexyl salicyate; gamma-dodecalactone; and, beta phenylethyl phenyl acetate.

Useful components of the perfume include materials of both natural and synthetic origin. They include single compounds and mixtures. Specific examples of such components may be found in the current literature, e.g., in Fenaroli's Handbook of Flavour Ingredients, 1975, CRC Press; Synthetic Food Adjuncts, 1947 by M. B. Jacobs, edited by Van Nostrand; or Perfume and Flavour Chemicals by S. Arctander 1969, Montclair, N.J. (USA).

It is commonplace for a plurality of perfume components to be present in a formulation. In the compositions of the present invention it is envisaged that there will be four or more, preferably five or more, more preferably six or more or even seven or more different perfume components.

In perfume mixtures preferably 15 to 25 wt.% are top notes. Top notes are defined by Poucher (Journal of the Society of Cosmetic Chemists 6(2):80 [1955]). Preferred top-notes are selected from citrus oils, linalool, linalyl acetate, lavender, dihydromyrcenol, rose oxide and cis-3-hexanol.

The International Fragrance Association has published a list of fragrance ingredients (perfumes) in 2011. (http://www.ifraorg.org/en-us/ingredients#.U7Z4hPIdWzk)

The Research Institute for Fragrance Materials provides a database of perfumes (fragrances) with safety information.

Perfume top note may be used to cue the whiteness and brightness benefit of the invention. Some or all of the perfume may be encapsulated, typical perfume components which it is advantageous to encapsulate, include those with a relatively low boiling point, preferably those with a boiling point of less than 300, preferably 100-250 Celsius. It is also advantageous to encapsulate perfume components which have a low CLog P (ie. those which will have a greater tendency to be partitioned into water), preferably with a CLog P of less than 3.0. These materials, of relatively low boiling point and relatively low CLog P have been called the "delayed blooming" perfume ingredients and include one or more of the following materials: allyl caproate, amyl acetate, amyl propionate, anisic aldehyde, anisole, benzaldehyde, benzyl acetate, benzyl acetone, benzyl alcohol, benzyl formate, benzyl iso valerate, benzyl propionate, beta gamma hexenol, camphor gum, laevo-carvone, d-carvone, cinnamic alcohol, cinamyl formate, cis-jasmone, cis-3-hexenyl acetate, cuminic alcohol, cyclal c, dimethyl benzyl carbinol, dimethyl benzyl carbinol acetate, ethyl acetate, ethyl aceto acetate, ethyl amyl ketone, ethyl benzoate, ethyl butyrate, ethyl hexyl ketone, ethyl phenyl acetate, eucalyptol, eugenol, fenchyl acetate, flor acetate (tricyclo decenyl acetate) , frutene (tricyclco decenyl propionate) , geraniol, hexenol, hexenyl acetate, hexyl acetate, hexyl formate, hydratropic alcohol, hydroxycitronellal, indone, isoamyl alcohol, iso menthone, isopulegyl acetate, isoquinolone, ligustral, linalool, linalool oxide, linalyl formate, menthone, menthyl acetphenone, methyl amyl ketone, methyl anthranilate, methyl benzoate, methyl benyl acetate, methyl eugenol, methyl heptenone, methyl heptine carbonate, methyl heptyl ketone, methyl hexyl ketone, methyl phenyl carbinyl acetate, methyl salicylate, methyl-n-methyl anthranilate, nerol, octalactone, octyl alcohol, p-cresol, p-cresol methyl ether, p-methoxy acetophenone, p-methyl acetophenone, phenoxy ethanol, phenyl acetaldehyde, phenyl ethyl acetate, phenyl ethyl alcohol, phenyl ethyl dimethyl carbinol, prenyl acetate, propyl bornate, pulegone, rose oxide, safrole, 4-terpinenol, alpha-terpinenol, and /or viridine. It is commonplace for a plurality of perfume components to be present in a formulation. In the compositions of the present invention it is envisaged that there will be four or more, preferably five or more, more preferably six or more or even seven or more different perfume components from the list given of delayed blooming perfumes given above present in the perfume.

Another group of perfumes with which the present invention can be applied are the so-called 'aromatherapy' materials. These include many components also used in perfumery, including components of essential oils such as Clary Sage, Eucalyptus, Geranium, Lavender, Mace Extract, Neroli, Nutmeg, Spearmint, Sweet Violet Leaf and Valerian.

It is preferred that the laundry treatment composition does not contain a peroxygen bleach, e.g., sodium percarbonate, sodium perborate, and peracid.

### Polymers

The composition may comprise one or more further polymers. Examples are carboxymethylcellulose, poly (ethylene glycol), poly(vinyl alcohol), polycarboxylates such as polyacrylates, maleic/acrylic acid copolymers and lauryl methacrylate/acrylic acid copolymers.

Where alkyl groups are sufficiently long to form branched or cyclic chains, the alkyl groups encompass branched, cyclic and linear alkyl chains. The alkyl groups are preferably linear or branched, most preferably linear.

### Adjunct Ingredients

The detergent compositions optionally include one or more laundry adjunct ingredients.

To prevent oxidation of the formulation an anti-oxidant may be present in the formulation.

The term "adjunct ingredient" includes: perfumes, dispersing agents, stabilizers, pH control agents, metal ion control agents, colorants, brighteners, dyes, odour control agent, pro-perfumes, cyclodextrin, perfume, solvents, soil release polymers, preservatives, antimicrobial agents, chlorine scavengers, anti-shrinkage agents, fabric crisping agents, spotting agents, antioxidants, anti-corrosion agents, bodying agents, drape and form control agents, smoothness agents, static control agents, wrinkle control agents, sanitization agents, disinfecting agents, germ control agents, mould control agents, mildew control agents, antiviral agents, antimicrobials, drying agents, stain resistance agents, soil release agents, malodour control agents, fabric refreshing agents, chlorine bleach odour control agents, dye fixatives, dye transfer inhibitors, shading dyes, colour maintenance agents, colour restoration, rejuvenation agents, anti-fading agents, whiteness enhancers, anti-abrasion agents, wear resistance agents, fabric integrity agents, anti-wear agents, and rinse aids, UV protection agents, sun fade inhibitors, insect repellents, anti-allergenic agents, enzymes, flame retardants, water proofing agents, fabric comfort agents, water conditioning agents, shrinkage resistance agents, stretch resistance agents, and combinations thereof. If present, such adjuncts can be used at a level of from 0.1% to 5% by weight of the composition

The invention will be further described with the following non-limiting examples.

### Examples

### Materials

Current commercial AES (Sodium alkyl ether sulfate) a mixture of C12/C14 alkyl with an average EO of ~3, the alkyl chain is generally palm kernel oil/coconut oil derived - comparative material.

Where r is a mixture of 10 and 12 in an approximate ratio of 3:1.

Narrow range AES (Sodium alkyl ether sulfate) C12-C14 alkyl with an average EO of ~3 - according to the invention.

Where r is 12.

The narrow range alkyl ethyl sulfate material according to the invention can be prepared as follows:
A calcium catalyst was prepared according to EP1747183, with the following composition: n-Butanol 73.5 wt.%, calcium hydroxide 15.2 wt. %, 2-ethylhexanoic acid, and 3.5 wt.%, conc. sulfuric acid 7.8 wt.%.

To prepare the catalyst, a three-neck round bottom flask is equipped with a magnetic stir bar, a glass stopper, a Dean-Stark trap filled with n-butanol, a condenser topped with a calcium chloride drying tube, and is placed in an oil bath. The n-butanol is charged to the flask and. stirring is initiated. The calcium hydroxide is slowly added, and allowed to stir for 15 minutes. A carboxylic acid (such as 2-ethylhexanoic acid) is then added to the mixture via syringe. The flask containing the mixture is then heated to above 120 degrees centigrade at atmospheric pressure. The stirring suspension is allowed to reflux for up to about 8 hours. Under these conditions, water and the dispersing medium will be removed during the process, but the dispersing medium is recycled into the reaction vessel. After cooling to room temperature, the stir bar is removed, and an overhead stirrer is added. The Dean-Stark trap, condenser, drying tube, oil bath, and stoppers are removed. A source of nitrogen, thermometer, water bath, and pressure equalizing dropping funnel are added. The pressure equalizing dropping funnel is charged with an inorganic acid (such as sulfuric acid), and the acid is added over the course of about 3 hours. The internal temperature is maintained at or below about 25 degrees centigrade by the use of a water bath and ice. After the acid is added completely, the suspension is allowed to stir for an additional 30-60 minutes at a temperature of about 25°C

This catalyst was used to produce narrow range ethoxylates.

915 g of a C14 alcohol (C14 = 100 wt.%) was charged into a 2 gallon stainless steel autoclave equipped with an overhead stirrer, internal steam heating, water cooling, and thermocouple. The C14 alcohol was vacuum dried at 90°C, then 2.1 g of catalyst was added and vacuum stripped at 90°C until all the solvent was removed (~ 5minutes). The reactor was heated to 140°C and ethylene oxide slowly added. After an induction period a small exothermic reaction is observed on which the addition of ethylene oxide is continued at a pressure of 2 bar, until 3 moles of ethylene oxide in total had been consumed. Temperature was controlled using water cooling and allowed to reach 180°C. When a mole ratio of 3:1 ethylene oxide to C14 alcohol had reacted to form alcohol ethoxylate the temperature was lowered to 90°C and the product vacuumed stripped for 3 hours.

The ethoxylation procedure can be alternatively repeated using a (C₁₁H₂₃COO)₂Ba described in Ind. Eng. Chem. Res. 1992, 31, 2419-2421 and a barium oxide/sulfuric acid catalyst as described in WO2012028435 (Kolb).

The ethoxylated alcohol was then sulfated as described earlier to produce an AES material according to the invention.

### Example 1 Comparing the ethoxylation distributions of current commercial AES material and AES material according to the invention

The ethoxylation profile of the ethoxylated material of the two surfactants was measured by Time of Flight (ToF) Mass Spectrometry. The conditions were as follows:
Samples are approximately 5ppm (as supplied) made with Methanol containing 10mM Ammonium Formate.

Samples were applied to the Mass Spec using a syringe pump set at 10ul/min.

Mass Spec was a Waters Xevo G2-XS Accurate Mass Quadrupole Time of Flight Mass Spectrometer (No mass correction).

Electrospray negative.

The settings for the mass spectrometry were as follows:
Polarity ES-
Analyser Sensitivity Mode
Capillary (kV) 1.0000
Sampling Cone 30.0000
Source Temperature (°C) 100
Source Offset 80°C
Desolvation Temperature (°C) 500
Cone Gas Flow (L/Hr) 10.0
Desolvation Gas Flow (L/Hr) 600.0

The results for the different ethoxylation (EO) materials in each sample were measured and normalized to 100% and shown in table 1. This allows for comparison of each sample as to the wt.% level of each EO level present compared to the total wt.% level of ethoxylated material.

**Table 1 - comparing wt.% of different EO materials in each sample**

| **EO** | **Commercial C12/C14 AES (SLES)** | **C14 Narrow range EO** |
|---|---|---|
| 1 | 29.7 | 18.1 |
| 2 | 25.6 | 19.8 |
| 3 | 17.2 | 23.6 |
| 4 | 11.0 | 17.7 |
| 5 | 7.0 | 10.8 |
| 6 | 4.0 | 6.1 |
| 7 | 2.6 | 2.7 |
| 8+ | 2.9 | 1.2 |

It is apparent that the commercial sample has an ethoxylation profile that is maximal for 1EO and drops off for each ascending EO degree. The material according to the invention has an ethoxylation profile that is lower in levels of 1EO and 2EO but has more 3EO and 4EO. It can be considered to be 'peaked' in the levels of 3EO and 4EO in comparison to the commercial material.

### Example 2 Viscosity measurements for formulations including current commercial AES

### material and AES material according to the invention

Four aqueous surfactant solutions were prepared so that the total amount of surfactant present was 15 wt.%. The composition of each solution is given in table 2, with the remainder water to 100 wt.%. Compositions according to the invention are denoted with numbers, comparative compositions with letters.

**Table 2 - Composition of Surfactant Solutions**

| **Sample** | **Sodium Linear Alkyl Benzene Sulphonate (LAS) wt.%** | **Commercial Sodium C12-14 3EO Alkyl Ether Sulphate (BR AES) wt.%** | **Sodium C14 3EO Alkyl Ether Sulphate (NR AES)** | **Coco amidopropyl betaine (CAPB)** |
|---|---|---|---|---|
| **A** | 3.75 | 11.25 | 0 | 0 |
| **1** | 3.75 | 0 | 11.25 | 0 |
| **B** | 3.375 | 10.125 | 0 | 1.5 |
| **2** | 3.375 | 0 | 10.125 | 1.5 |

The viscosity of each solution was measured as a function of salt content, the appropriate amount of sodium chloride was added to a sub sample of each composition. The viscosity of each solution was measured at a shear rate of 1.94 s⁻¹ using an Anton Paar rheometer with cup and bob methodology at a temperature of 25 ⁰C. The concentration of surfactant was maintained at 15 wt.%. The results are illustrated in table 3.

**Table 3 - Maximum viscosity and required NaCl level for samples A, B, 1 and 2.**

| **Sample** | **Maximum Viscosity (cP)** | **% NaCl to achieve a viscosity of 10,000 cP** |
|---|---|---|
| **A** | 11,500.00 | 3.8 |
| **1** | 63,100.00 | 1.2 |
| **B** | 17,200.00 | 1.4 |
| **2** | 34,900.00 | 0.4 |

This data shows that the narrow range alkyl ether sulphate materials according to the invention generate significantly higher maximum viscosities as well as requiring lower level of sodium chloride to increase the sample viscosity.

## Claims

1. A liquid detergent composition comprising:
from 2 to 25 wt.% of a C12-C14 alkyl ethoxylated sulfate surfactant;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24 wt.%, the level of 3EO is from 20 to 35 wt.%, and the level of 4EO is from 12 to 25 wt.%; and,
wherein the C12-C14 alkyl ethoxylated sulfate surfactant includes at most 10 wt.% alkyl chains of C15 and higher.

2. A detergent composition according to claim 1, wherein the alkyl ethoxylated sulfate surfactant comprises a C14 alkyl group at a level of at least 75 wt.%, even more preferably at least 80 wt.%, even more preferably at least 85 wt.%, even more preferably at least 90 wt.%, even more preferably at least 95 wt.% of the alkyl ethoxylated sulfate surfactant.

3. A detergent composition according to claim 1 or claim 2, wherein the alkyl ethoxylated sulfate surfactant is present at a level of from 2.5 to 20 wt.%.

4. A detergent composition according to any preceding claim, wherein the average degree of ethoxylation (EO) is from 2.7 to 3.3.

5. A detergent composition according to any preceding claim, wherein with reference to the wt.% of the total ethoxylated portion of said alkyl ethoxylated sulfate surfactant, the level of 1EO is from 13 to 22 wt.%, more preferably from 14 to 21 wt.%, even more preferably from 15 to 20 wt.%.

6. A detergent composition according to any preceding claim, wherein with reference to the wt.% of the total ethoxylated portion of said alkyl ethoxylated sulfate surfactant, the level of 2EO is from 16 to 23 wt.%, preferably from 17 to 22 wt.%, more preferably from 18 to 22 wt.%.

7. A detergent composition according to any preceding claim, wherein with reference to the wt.% of the total ethoxylated portion of said alkyl ethoxylated sulfate surfactant, the level of 3EO is from 20 to 30 wt.%, preferably from 21 to 28 wt.%, more preferably from 22 to 26 wt.%.

8. A detergent composition according to any preceding claim, wherein with reference to the wt.% of the total ethoxylated portion of said alkyl ethoxylated sulfate surfactant, the level of 4EO is from 13 to 24 wt.%, preferably from 14 to 22 wt.%, more preferably from 15 to 21 wt.%.

9. A detergent composition according to any preceding claim, additionally comprising from 1 to 40 wt.%, preferably from 2 to 30 wt.%, more preferably from 4 to 25 wt.%, most preferably from 5 to 20 wt.% of one or more other surfactants selected from anionic surfactants, nonionic surfactants, cationic surfactants and amphoteric surfactants, preferably anionic surfactants, nonionic surfactants and amphoteric surfactants.

10. A detergent composition according to any preceding claim, wherein the composition is a laundry liquid detergent composition or a liquid hand dish wash composition, more preferably an aqueous liquid detergent composition, even more preferably an aqueous laundry liquid detergent composition or an aqueous liquid hand dish wash composition.

11. Use of a C12-C14 alkyl ethoxylated sulfate surfactant to increase the viscosity of a liquid detergent composition;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24 wt.%, the level of 3EO is from 20 to 35 wt.%, and the level of 4EO is from 12 to 25 wt.%; and,
wherein the C12-C14 alkyl ethoxylated sulfate surfactant includes at most 10 wt.% alkyl chains of C15 and higher.

12. Method to increase viscosity of a liquid detergent composition, wherein said method involves inclusion of from 2 to 25 wt.% of a C12-C14 alkyl ethoxylated sulfate surfactant;
wherein the alkyl ethoxylated sulfate surfactant comprises a C14 alkyl group at a level of at least 70 wt.% of the alkyl ethoxylated sulfate surfactant;
wherein the average degree of ethoxylation (EO) is from 2.5 to 3.5;
wherein with reference to the wt.% of the total ethoxylated portion of said alkyl ethoxylated sulfate surfactant, the level of 1EO is from 12 to 23 wt.%, the level of 2EO is from 15 to 24 wt.%, the level of 3EO is from 20 to 35 wt.%, and the level of 4EO is from 12 to 25 wt.%; and,
wherein the C12-C14 alkyl ethoxylated sulfate surfactant includes at most 10 wt.% alkyl chains of C15 and higher.

13. Use according to claim 11, or method according to claim 12, wherein said use or method to increase viscosity is made in reference to a constant salt level, preferably NaCl, in said detergent composition.

## Patentansprüche

1. Flüssige Waschmittelzusammensetzung, umfassend:
2 bis 25 Gew.-% eines ethoxylierten C12-C14-Alkylsulfat-Tensids;
wobei das ethoxylierte Alkylsulfat-Tensid eine C14-Alkylgruppe in einer Menge von mindestens 70 Gew.-% des ethoxylierten Alkylsulfat-Tensids umfasst;
wobei der durchschnittliche Ethoxylierungsgrad (EO) 2,5 bis 3,5 beträgt;
wobei in Bezug auf die Gew.-% des gesamten ethoxylierten Anteils des ethoxylierten Alkylsulfat-Tensids der Anteil von 1 EO 12 bis 23 Gew.-%, der Anteil von 2EO 15 bis 24 Gew.-%, der Anteil von 3 EO 20 bis 35 Gew.-% und der Anteil von 4EO 12 bis 25 Gew.-% beträgt; und
wobei das ethoxylierte C12-C14-Alkylsulfat-Tensid höchstens 10 Gew.-% Alkylketten von C15 und höher umfasst.

2. Waschmittelzusammensetzung nach Anspruch 1, wobei das ethoxylierte Alkylsulfat-Tensid eine C14-Alkylgruppe in einer Menge von mindestens 75 Gew.-%, noch bevorzugter von mindestens 80 Gew.-%, noch bevorzugter von mindestens 85 Gew.-%, noch bevorzugter von mindestens 90 Gew.-%, noch bevorzugter von mindestens 95 Gew.-% des ethoxylierten Alkylsulfat-Tensids umfasst.

3. Waschmittelzusammensetzung nach Anspruch 1 oder Anspruch 2, wobei das ethoxylierte Alkylsulfat-Tensid in einer Menge von 2,5 bis 20 Gew.-% vorliegt.

4. Waschmittelzusammensetzung nach einem vorhergehenden Anspruch, wobei der durchschnittliche Ethoxylierungsgrad (EO) 2,7 bis 3,3 beträgt.

5. Waschmittelzusammensetzung nach einem vorhergehenden Anspruch, wobei in Bezug auf die Gew.-% des gesamten ethoxylierten Anteils des ethoxylierten Alkylsulfat-Tensids der Anteil von 1 EO 13 bis 22 Gew.-%, bevorzugter 14 bis 21 Gew.-%, noch bevorzugter 15 bis 20 Gew.-% beträgt.

6. Waschmittelzusammensetzung nach einem vorhergehenden Anspruch, wobei in Bezug auf die Gew.-% des gesamten ethoxylierten Anteils des ethoxylierten Alkylsulfat-Tensids der Anteil von 2 EO 16 bis 23 Gew.-%, bevorzugt 17 bis 22 Gew.-%, bevorzugter 18 bis 22 Gew.-% beträgt.

7. Waschmittelzusammensetzung nach einem vorhergehenden Anspruch, wobei in Bezug auf die Gew.-% des gesamten ethoxylierten Anteils des ethoxylierten Alkylsulfat-Tensids der Anteil von 3 EO 20 bis 30 Gew.-%, bevorzugt 21 bis 28 Gew.-%, bevorzugter 22 bis 26 Gew.-% beträgt.

8. Waschmittelzusammensetzung nach einem vorhergehenden Anspruch, wobei in Bezug auf die Gew.-% des gesamten ethoxylierten Anteils des ethoxylierten Alkylsulfat-Tensids der Anteil von 4 EO 13 bis 24 Gew.-%, bevorzugt 14 bis 22 Gew.-%, bevorzugter 15 bis 21 Gew.-% beträgt.

9. Waschmittelzusammensetzung nach einem vorhergehenden Anspruch, zusätzlich umfassend 1 bis 40 Gew.-%, bevorzugt 2 bis 30 Gew.-%, bevorzugter 4 bis 25 Gew.-%, höchst bevorzugt 5 bis 20 Gew.-% eines oder mehrerer anderer Tenside, ausgewählt unter anionischen Tensiden, nichtionischen Tensiden, kationischen Tensiden und amphoteren Tensiden, bevorzugt anionischen Tensiden, nichtionischen Tensiden und amphoteren Tensiden.

10. Waschmittelzusammensetzung nach einem vorhergehenden Anspruch, wobei die Zusammensetzung eine flüssige Wäschewaschmittelzusammensetzung oder eine flüssige Handgeschirrspülzusammensetzung, bevorzugter eine flüssige wässrige Waschmittelzusammensetzung, noch bevorzugter eine flüssige wässrige Wäschewaschmittelzusammensetzung oder eine flüssige wässrige Handspülzusammensetzung ist.

11. Verwendung eines ethoxylierten C12-C14-Alkylsulfat-Tensids zur Erhöhung der Viskosität einer flüssigen Waschmittelzusammensetzung;
wobei das ethoxylierte Alkylsulfat-Tensid eine C14-Alkylgruppe in einem Anteil von mindestens 70 Gew.-% des ethoxylierten Alkylsulfat-Tensids umfasst;
wobei der durchschnittliche Ethoxylierungsgrad (EO) 2,5 bis 3,5 beträgt;
wobei in Bezug auf die Gew.-% des gesamten ethoxylierten Anteils des ethoxylierten Alkylsulfat-Tensids der Anteil von 1 EO 12 bis 23 Gew.-%, der Anteil von 2 EO 15 bis 24 Gew.-%, der Anteil von 3 EO 20 bis 35 Gew.-% und der Anteil von 4 EO 12 bis 25 Gew.-% beträgt; und
wobei das ethoxylierte C12-C14-Alkylsulfat-Tensid höchstens 10 Gew.-% Alkylketten von C15 und höher umfasst.

12. Verfahren zur Erhöhung der Viskosität einer flüssigen Waschmittelzusammensetzung, wobei das Verfahren den Einbezug von 2 bis 25 Gew.-% eines ethoxylierten C12-C14-Alkylsulfat-Tensids umfasst;
wobei das ethoxylierte Alkylsulfat-Tensid eine C14-Alkylgruppe in einem Anteil von mindestens 70 Gew.-% des ethoxylierten Alkylsulfat-Tensids umfasst;
wobei der durchschnittliche Ethoxylierungsgrad (EO) 2,5 bis 3,5 beträgt; und wobei in Bezug auf die Gew.-% des gesamten ethoxylierten Anteils des ethoxylierten Alkylsulfat-Tensids der Anteil von 1 EO 12 bis 23 Gew.-%, der Anteil von 2 EO 15 bis 24 Gew.-%, der Anteil von 3 EO 20 bis 35 Gew.-% und der Anteil von 4 EO 12 bis 25 Gew.-% beträgt; und
wobei das ethoxylierte C12-C14-Alkylsulfat-Tensid höchstens 10 Gew.-% Alkylketten von C15 und höher einschließt.

13. Verwendung nach Anspruch 11 oder Verfahren nach Anspruch 12, wobei die Verwendung oder das Verfahren zur Erhöhung der Viskosität in Bezug auf einen konstanten Salzgehalt, bevorzugt NaCl, in der Waschmittelzusammensetzung erfolgt.

## Revendications

1. Composition détergente liquide comprenant :
2 à 25 % en poids d'un tensioactif alkylsulfate en C12-C14 éthoxylé ; dans laquelle le tensioactif alkylsulfate éthoxylé comprend un groupe alkyle en C14 à raison d'au moins 70 % en poids du tensioactif alkylsulfate éthoxylé ;
dans laquelle le degré moyen d'éthoxylation (EO) est de 2,5 à 3,5 ;
dans laquelle, en référence au pourcentage en poids de la portion éthoxylée totale dudit tensioactif alkylsulfate éthoxylé, le niveau de 1EO est de 12 à 23 % en poids, le niveau de 2EO est de 15 à 24 % en poids, le niveau de 3EO est de 20 à 35 % en poids, et le niveau de 4EO est de 12 à 25 % en poids ; et
dans laquelle le tensioactif alkylsulfate éthoxylé en C12-C14 contient au plus 10 % en poids de chaînes alkyle en C15 et plus.

2. Composition détergente selon la revendication 1, dans laquelle le tensioactif alkylsulfate éthoxylé comprend un groupe alkyle en C14 à raison d'au moins 75 % en poids, mieux encore d'au moins 80 % en poids, mieux encore d'au moins 85 % en poids, mieux encore d'au moins 90 % en poids, mieux encore d'au moins 95 % en poids du tensioactif alkylsulfate éthoxylé.

3. Composition détergente selon la revendication 1 ou 2, dans laquelle le tensioactif alkylsulfate éthoxylé est présent à raison de 2,5 à 20 % en poids.

4. Composition détergente selon l'une quelconque des revendications précédentes, dans laquelle le degré moyen d'éthoxylation (EO) est de 2,7 à 3,3.

5. Composition détergente selon l'une quelconque des revendications précédentes, dans laquelle, en référence au pourcentage en poids de la portion éthoxylée totale dudit tensioactif alkylsulfate éthoxylé, le niveau de 1EO est de 13 à 22 % en poids, mieux encore de 14 à 21 % en poids, plus particulièrement de 15 à 20 % en poids.

6. Composition détergente selon l'une quelconque des revendications précédentes, dans laquelle, en référence au pourcentage en poids de la portion éthoxylée totale dudit tensioactif alkylsulfate éthoxylé, le niveau de 2EO est de 16 à 23 % en poids, de préférence de 17 à 22 % en poids, mieux encore de 18 à 22 % en poids.

7. Composition détergente selon l'une quelconque des revendications précédentes, dans laquelle, en référence au pourcentage en poids de la portion éthoxylée totale dudit tensioactif alkylsulfate éthoxylé, le niveau de 3EO est de 20 à 30 % en poids, de préférence de 21 à 28 % en poids, mieux encore de 22 à 26 % en poids.

8. Composition détergente selon l'une quelconque des revendications précédentes, dans laquelle, en référence au pourcentage en poids de la portion éthoxylée totale dudit tensioactif alkylsulfate éthoxylé, le niveau de 4EO est de 13 à 24 % en poids, de préférence de 14 à 22 % en poids, mieux encore de 15 à 21 % en poids.

9. Composition détergente selon l'une quelconque des revendications précédentes, comprenant de plus 1 à 40 % en poids, de préférence 2 à 30 % en poids, mieux encore 4 à 25 % en poids, tout spécialement 5 à 20 % en poids d'un ou plusieurs autres tensioactifs choisis parmi les tensioactifs anioniques, les tensioactifs non-ioniques, les tensioactifs cationiques et les tensioactifs amphotères, de préférence les tensioactifs anioniques, les tensioactifs non-ioniques et les tensioactifs amphotères.

10. Composition détergente selon l'une quelconque des revendications précédentes, laquelle composition est une composition détergente liquide pour le linge ou une composition liquide pour le lavage de la vaisselle à la main, mieux encore une composition détergente liquide aqueuse, plus particulièrement une composition détergente liquide aqueuse pour le linge ou une composition liquide aqueuse pour le lavage de la vaisselle à la main.

11. Utilisation d'un tensioactif alkylsulfate éthoxylé en C12-C14 pour augmenter la viscosité d'une composition détergente liquide ;
dans laquelle le tensioactif alkylsulfate éthoxylé comprend un groupe alkyle en C14 à raison d'au moins 70 % en poids du tensioactif alkylsulfate éthoxylé ;
dans laquelle le degré moyen d'éthoxylation (EO) est de 2,5 à 3,5 ;
dans laquelle, en référence au pourcentage en poids de la portion éthoxylée totale dudit tensioactif alkylsulfate éthoxylé, le niveau de 1EO est de 12 à 23 % en poids, le niveau de 2EO est de 15 à 24 % en poids, le niveau de 3EO est de 20 à 35 % en poids, et le niveau de 4EO est de 12 à 25 % en poids ; et
dans laquelle le tensioactif alkylsulfate éthoxylé en C12-C14 contient au plus 10 % en poids de chaînes alkyle en C15 et plus.

12. Procédé pour augmenter la viscosité d'une composition détergente liquide, lequel procédé implique l'incorporation de 2 à 25 % en poids d'un tensioactif alkylsulfate éthoxylé en C12-C14 ;
dans lequel le tensioactif alkylsulfate éthoxylé comprend un groupe alkyle en C14 à raison d'au moins 70 % en poids du tensioactif alkylsulfate éthoxylé ;
dans lequel le degré moyen d'éthoxylation (EO) est de 2,5 à 3,5 ;
dans lequel, en référence au pourcentage en poids de la portion éthoxylée totale dudit tensioactif alkylsulfate éthoxylé, le niveau de 1EO est de 12 à 23 % en poids, le niveau de 2EO est de 15 à 24 % en poids, le niveau de 3EO est de 20 à 35 % en poids, et le niveau de 4EO est de 12 à 25 % en poids ; et
dans lequel le tensioactif alkylsulfate éthoxylé en C12-C14 contient au plus 10 % en poids de chaînes alkyle en C15 et plus.

13. Utilisation selon la revendication 11, ou procédé selon la revendication 12, laquelle utilisation ou lequel procédé pour augmenter la viscosité est mis en œuvre en référence à un niveau de sel, de préférence NaCl, constant, dans ladite composition détergente.
